

## UNITED STATES PATENT OFFICE

1,934,305

METHOD FOR THE PREPARATION OF ZINC  
SULPHATE SOLUTIONS

William Henry Hannay and Frederick Eric Lee,  
Trail, British Columbia, Canada, assignors to  
The Consolidated Mining and Smelting Com-  
pany of Canada, Limited, Montreal, Quebec,  
Canada, a corporation of Canada

No Drawing. Application November 28, 1931  
Serial No. 577,860

2 Claims. (CL. 204—18)

Our invention relates to a method of preparing zinc sulphate solutions for hydro-metallurgical operations, characterized by the step of adjusting the amount of cobalt to the free acid in 5 the solution for inhibiting corrosion and disintegration of the anode and the entrainment of lead in the deposited zinc without causing resolution effects or preventing the deposit of coherent reguline zinc.

10 Complex zinc ores usually contain cobalt, and previous investigators have postulated that its presence in sulphate solutions, even in the most minute quantities, causes resolution effects and prevents the deposition of coherent reguline zinc, 15 and on that hypothesis the solution, heretofore, has been highly purified to completely eliminate it.

We found, however, that when a lead anode is used in the electrolysis of such solutions the zinc 20 deposited at the cathode contained lead detached from the anode by corrosion, and that the corrosion is largely, if not wholly, due to the absence of cobalt in the electrolyte.

The useful life of the lead anode in the electrolysis of a sulphate solution in which there is 25 no cobalt present does not average more than three months and when it is present in the solution its useful life averages about three years. When the amount of cobalt is properly adjusted 30 to the free acid of the solution there is neither corrosion of the anode nor lead in the zinc and no resolution effects to prevent the deposit of coherent reguline zinc.

The optimum amount of cobalt in the solution 35 according to this adjustment, is maintained between 4 and 6 milligrams per litre containing approximately 10% free sulphuric acid and up to 15 milligrams of cobalt per litre in sulphate solutions containing 7 or 8% free acid. Amounts be- 40 low these ratios have no material beneficial re-

sults, while amounts in excess of them impair the efficiency of the cell at a correspondingly increasing rate in proportion to the increase of cobalt. A constant balance between the cobalt and the free acid of the solution must therefore be maintained either by purifying the solution when the cobalt fraction exceeds the correct ratio, or by adding cobalt when it is necessary to bring it up to that ratio, and this balance is an important factor governing the cost of production and sale price of the zinc, particularly in the operation of large zinc extraction plants, having several thousand lead anodes in constant use.

Having thus fully described our invention, what we claim as new and desire to secure by Letters Patent is:

1. A hydro-metallurgical method for the electrolytic deposition of zinc from a sulphate solution which comprises, when using a lead anode in the electrolysis, the step of incorporating cobalt in the solution in the proportion of from 4 to 6 milligrams of cobalt per litre of solution containing approximately 10% free acid, and thereafter maintaining said specified ratio balance either by purification of the solution under treatment or by increasing the cobalt content.

2. A hydro-metallurgical method for the electrolytic deposition of zinc from a sulphate solution when using a lead anode which comprises maintaining the cobalt-acid ratio in the solution under treatment within such limits that at no time does the cobalt content recede below a minimum of from 4 to 6 milligrams per litre of solution containing 10% free acid solution or exceed a maximum of 15 milligrams per litre of solution containing 7 to 8% free acid.

WILLIAM HENRY HANNAY.  
FREDERICK ERIC LEE.

95